# EUROPEAN PATENT APPLICATION

(11) **EP 1 160 371 A1**
(43) Date of publication of application: **05.12.2001**
(21) Application number: 99923997.3
(22) Date of filing: 10.06.1999
(51) Int. Cl.: D06M 15/59, D06M 15/564, D06N 3/14, C08L 77/00, C08L 75/04

(54) **FIBER TREATING AGENT AND FIBER TREATED WITH THE SAME**

(30) Priority: 12.06.1998 JP 18146498
(71) Applicant: MATSUMOTO YUSHI-SEIYAKU CO., LTD., Yao-shi, Osaka 581-0075 (JP)
(72) Inventor: HIZUMI, Nanae, Matsumoto Yushi-Seiyaku Co. Ltd., Yao-shi, Osaka 581-0075 (JP); NOMURA, Yasuyuki, Matsumoto Yushi-Seiyaku Co. Ltd., Yao-shi, Osaka 581-0075 (JP); DOI, Tetsuo, Matsumoto Yushi-Seiyaku Co. Ltd., Yao-shi, Osaka 581-0075 (JP)
(74) Representative: Cresswell, Thomas Anthony
(86) International application number: JP9903110
(87) International publication number: WO9964663

(57) **Abstract**

A fiber finish which prevents the emission of snow on the surface of polyamide fibers and the like during long-term storage so as to prevent fluffs, ends down and decreased knit fabric quality in down-stream processes caused by the snow, and imparts high cohesion to synthetic filament. The finish contains (a) a urethane compound produced in the reaction of a polyhydric alcohol having 12 or more carbon atoms and an organic diisocyanate, or (b) an amide compound produced in the reaction of a polycarboxylic acid having 12 or more carbon atoms and an organic diisocyanate. Above all, the urethane compound produced in the reaction of a dimeric alcohol having a molecular weight of 300 to 1,000 and an organic diisocyanate, and the amide compound produced in the reaction of a dimeric acid having a molecular weight of 300 to 1,000 and an organic diisocyanate are preferable.

## Description

### Technical Field

The present invention relates to a fiber finish and fiber applied with the same. Specifically, the present invention relates to a fiber finish, which imparts high cohesion to synthetic filament and prevents the emission of oligomer and polymer additives from polyamide fiber or polyamide fiber-covered yarn during long-term storage, and fiber treated with the same.

### Technical Background

The production process of synthetic fibers such as nylon 6, nylon 66 and polyester fiber, specifically the production process of synthetic filaments, has been rationalized by cutting several production steps, and their production efficiency has been improved by increasing operation speed. Polyamide fiber, such as nylon 6 and nylon 66 fiber, produced in POY (pre-oriented yarn) system with about 4,000 m/min take-up speed or in high-speed spinning system with 5,000 m/min or more take-up speed emits oligomer on its surface during storage. And the emitted oligomer (called snow) deposits on the bodies (for example, guides, rollers, and heaters) to which fiber contacts in down-stream process, and increases the friction between yarn and contact surface to cause damage on fiber and increase fluffs or ends down.

Polyurethane yarn covered with polyamide fiber is fed to the knitting process for producing hosiery called support panty hose, of which demand has been increasing recently. The polyurethane yarn covered with polyamide fiber (hereinafter referred to as covered yarn) also emits polyamide oligomer, urethane oligomer and additives in polyurethane fiber polymer onto its surface during storage, and bears some troubles, such as increased ends down or low fabric quality in knitting process due to increased friction on yarn caused from the deposited snow on guides or needles.

Those troubles are often found on polyamide fiber produced in POY system or high-speed spinning system, or especially on high-multi-filament yarn, which has large surface area. Thus there has been strong demand for a fiber finish which prevents snow generation on polyamide fiber or polyurethane yarn covered with polyamide fiber during long term storage in order to improve the processing performance of those fiber and yarn in down-stream process and the quality of resultant knit fabric.

Fiber finishes for polyester and polyamide filament are usually applied to fiber in spinning process from an aqueous emulsion of 3-30 % finish concentration. Finish-applied fiber is further processed in 2-step system, such as conventional (UDY-DT) system, POY-DT system and POY-DTY system, where extruded filament is taken up and then drawn or draw-twisted; or in 1-step system, such as spin-draw system where filament is continuously extruded, drawn and taken up, and high-speed spinning system where filament is taken up without drawing operation.

For preventing cross yarn or loops on yarn packages and for improving processability in down-stream process, filament yarn is intermingled to be imparted with cohesion at an interlacer before take-up. With the increase of yarn production speed, sufficient intermingling of filament at an interlacer becomes more difficult, and excessively high-pressure air is sometimes fed to an interlacer for intermingling filament resulting in fluffs and ends down caused from high-pressure air.

For solving such troubles, a finish imparting sufficient filament cohesion has been greatly demanded.

### Disclosure of Invention

The object of the present invention is to provide a fiber finish.

Another object of the present invention is to provide a fiber finish, which is effective to prevent the emission of oligomer or polymer additives from synthetic fiber, such as polyamide fiber, during long term storage.

Still another object of the present invention is to provide a fiber finish which prevents fluffs, ends down or poor knit fabric quality in down-stream process by preventing snow generation caused from oligomer or polymer additives.

Further object of the present invention is to provide a fiber finish which imparts high cohesion to synthetic fiber.

Still further object of the present invention is to provide synthetic fiber applied with a fiber finish of the present invention, which has high cohesion and generates little snow not to result in fluffs, ends down and low knit fabric quality.

And still further object and advantage of the present invention is illustrated in the following description.

According to the present invention, the above object and the advantage of the present invention is achieved, first, with a fiber finish characterized by containing at least one compound selected from a group consisting of urethane compounds which are the reaction products of polyhydric alcohol having 12 or more carbon atoms and organic diisocyanate; and amide compounds which are the reaction products of polycarboxylic acid having 12 or more carbon atoms and organic diisocyanate.

According to the present invention, the above object and the advantage of the present invention is achieved, secondly, by the synthetic fiber applied with the fiber finish of the present invention.

According to the present invention, in addition, the above object and advantage of the present invention is achieved, thirdly, by applying at least one compound selected from a group consisting of urethane compounds which are the reaction products of polyhydric alcohol having 12 or more carbon atoms and organic diisocyanate, and amide compounds which are the reaction products of polycarboxylic acid having 12 or more carbon atoms and organic diisocyanate to a fiber finish.

### Detailed Description of Invention

The urethane compounds employed in the present invention are produced by reacting a polyhydric alcohol with an organic diisocyanate.

The polyhydric alcohols are those having 12 or more carbon atoms, preferably those having 12-60 carbon atoms, more preferably those having 20-40 carbon atoms, such as diol.

The examples of the polyhydric alcohols are alkylene diols, such as dodecamethylene diol and octadecamethylene diol, dimeric alcohols produced by reducing dimeric acids derived from unsaturated fatty acids, and polyoxyalkylene polyhydric alcohols produced by adding ethylene oxide or propylene oxide to the said alkylene diols or dimeric alcohols. One or more of those are applied to the finish of the present invention.

The examples of organic diisocyanates applied to the present invention are tolylene diisocyanate, 1,3-bis(isocyanate methyl) cyclohexane, hexamethylene diisocyanate, octadecamethylene diisocyanate, dicyclohexylmethane-4,4 diisocyanate, and the like. One or more of them are applied to the finish of the present invention.

The amide compounds applicable to the present invention are the reaction products of polycarboxylic acid and organic diisocyanate in a reaction with decarboxylation.

Preferable polycarboxylic acids for the above reaction are polycarboxylic acids having 12 or more carbon atoms, preferably from 12 to 60 carbon atoms, and more preferably dicarboxylic acids of 300 to 1000 molecular weight, such as dimeric acid produced by dimerizing unsaturated fatty acid.

The above polycarboxylic acids are alkylene dicarboxylic acids, such as dodecamethylene dicarboxylic acid and octadecamethylene dicarboxylic acid; alkenyl succinic acids, such as dodecenyl succinic acid and octadecenyl succinic acid; and dimeric acids produced by dimerizing unsaturated fatty acids, for example, linoleic acid. One or more of them are fed to the reaction.

In addition, an aromatic carboxylic acid having less than 12 carbon atoms, such as phthalic acid, isophthalic acid or telephthalic acid can be applied simultaneously with the said polycarboxylic acids having 12 or more carbon atoms.

Such aromatic dicarboxylic acid is used by 1 mole or less, preferably by 0.5 mole, per 1 mole of the above polycarboxylic acid.

The organic diisocyanates applicable to the above reaction are the same as those described above.

It is preferable to feed the polyhydric alcohol or polycarboxylic acid to organic diisocyanate in a stoichiometrically excessive ratio in the reaction for producing the above-mentioned urethane or amide compound to produce a urethane or amide compound having 800 to 30,000 molecular weight, more preferably, 1,000 to 10,000 molecular weight.

Urethane or amide compounds having more than 30,000 molecular weight have poor compatibility to other components of a fiber finish. On the other hand, urethane or amide compounds of less than 800 molecular weight are not effective to prevent the emission of polyamide oligomer from polyamide fiber during storage, and not effective to impart cohesion to synthetic filament.

Polyhydric alcohols or polycarboxylic acids having less than 12 carbon atoms produce a urethane compound having poor compatibility to other components in a fiber finish and being less effective for preventing the emission of amide oligomer from polyamide fiber or urethane oligomer from polyurethane fiber during storage. For producing a compound which is compatible enough to other components in a fiber finish and effective to prevent the emission of amide or urethane oligomer, and imparts cohesion to fiber, dimeric acids having 300 to 1,000 molecular weight are preferable as the polycarboxylic acid, and dimeric alcohols produced by reducing those dimeric acids are preferable as the polyhydric alcohol.

The preferable stoichiometric ratio of the polyhydric alcohol or polycarboxylic acid to that of the organic diisocyanate for their reaction is 2 to 10 equivalent weight to 1 equivalent weight.

Less than 2 equivalent weight of a polyhydric alcohol or polycarboxylic acid results in a urethane or amide compound having high molecular weight and poor compatibility to other components in a fiber finish. And more than 10 equivalent weight of a polyhydric alcohol or polycarboxylic acid results in a urethane or amide compound having poor effect to prevent amide oligomer emission from polyamide fiber.

The terminals of the amide compound of the present invention can be partially or wholly neutralized with alkali metals or alkalis such as ammonia, amine, or alkanol amine, in the case that the terminals are carboxyl groups.

The urethane compound of the present invention includes urethane compounds of which molecules contain amide structure produced by substituting less than 50-mole % of a polyhydric alcohol with a polycarboxylic acid.

In addition, the amide compounds of the present invention include amide compounds of which molecule contain urethane structure produced by substituting less than 50-mole % of polycarboxylic acid with polyhydric alcohol.

The above-mentioned urethane compounds having amide structure and the amide compounds having urethane structure can also be applied to the finish of the present invention in the same manner as the urethane compounds and amide compounds described before.

The urethane compounds and amide compounds in the present invention can be produced by reacting an organic diisocyanate with a polyhydric alcohol, a polycarboxylic acid, or the mixture of them at 50 - 180 °C.

One of the above-mentioned urethane compounds and amide compounds or the complex compounds of those compounds can be used as the fiber finish of the present invention. And other known components generally blended in fiber finishes, such as lubricants including aliphatic esters, mineral oils and EO/PO polyethers; nonionic emulsifiers including polyoxyethylene alkylethers, polyoxyethylene alkylarylethers, PEG fatty acid esters, polyhydric alcohol esters and polyoxyethylene polyhydric alcohol esters; and antistatic agents including alkali metal salts, for example, alkane sulfonates and alkyl phosphates, amine salts, alkylimidazoline surfactants, and betaine surfactants. The components often blended are aliphatic esters, such as dodecyl stearate, isooctyl palmitate and isopropyl palmitate, and polyoxyethylene alkylethers.

The fiber finish of the present invention contains 0.5 - 80 weight percent, preferably 2 - 30 weight percent, of the urethane compounds and/or amide compounds mentioned above.

The application procedure of the finish of the present invention to fiber consists of dissolving the urethane compounds and/or amide compounds in base oil (neat finish), organic solvent, or low-viscosity mineral oil to make a dilution, or in water to make an emulsion; and applying the dilution or emulsion to fiber in spinning, drawing, false-twist texturing, rewinding, or warp preparation process with a known application system, such as kiss-roll application, metering pump application, spray or dipping. The pickup of the above urethane or amide compound is 0.01 - 3.0 weight percent, preferably 0.02 - 1.0 weight percent of fiber weight. In most cases, 15 - 90 weight percent of lubricants and 5 - 50 weight percent of nonionic emulsifiers are blended to a fiber finish.

Thus the present invention provides the synthetic fibers, such as polyamide and polyurethane fibers, and covered yarn produced by covering polyurethane fiber with polyamide fiber, which are applied with the fiber finish of the present invention.

The present invention also provides the application of urethane and amide compounds to a fiber finish, which has not been known in the conventional finish technology.

The following examples describe the present invention in detail, though the present invention is not restricted within the scope of those examples.

### Example 1

The fiber finishes of the present invention 1 to 8 and the comparative fiber finishes 9 - 11 in Table 3, which were formulated by blending a given amount of the compounds in Table 1 with the standard finish A in Table 2, were made into aqueous emulsion. The aqueous emulsions of those finishes were applied to a deoiled Nylon 66 multifilament yarn (50d/13f) in an amount at which solid matter in a finish emulsion was applied in 1 % of fiber weight. The cohesion and oligomer emission under accelerated aging condition of the yarn samples applied with the finishes were tested. The result is shown in Table 3.

The tests were carried out in the following procedure.

### (1) Cohesion

The top end of a yarn sample of 30 cm long was fixed and a 30-g loading was hanged on the bottom end. The point at 15-cm distant from top end was cut with a pair of sharp scissors and the length of separated filament (fluff length) was measured and represented by millimeters. Smaller value indicates better cohesion of yarn.

### (2) Oligomer emission

A yarn sample wound on a cone was stored in an incubator at 50 ° C and 90 %RH for a week. After the storage the yarn sample was driven on black velvet at 200 m/min for 5 minutes. The snow (polyamide oligomer) deposited on the velvet was visually inspected.

### Standard of evaluation

ⓞ : no snow deposit ○: a little snow deposit Δ: more snow deposit

×: a lot of snow deposit × ×: extremely much snow deposit

### Example 2

The compounds A, B and D shown in Table 1 was blended in the standard finish B shown in Table 4 to prepare the finishes of the present invention Nos. 12 to 16 and the comparative finishes Nos. 17 and 18 shown in Table 5. Those finishes were applied neat to nylon 66 filament yarn (10d/7f), polyurethane yarn (20d/2f) and a covered yarn produced of those yarns to dress the yarns with 2 weight percent of fiber weight of solid component of the finishes, and tested. A yarn sample without those finishes and an after oil was simultaneously tested. The result is shown in Table 5.

### (3) Polymer additive emission

The polyurethane yarn and covered yarn samples were stored in a freezer at 0 °C for one month and snow (polymer additive in the polyurethane yarn) deposited on yarn surface was inspected by taking electron microphotograph.

### Standard of evaluation

ⓞ: no snow deposit ○: a little snow deposit Δ: more snow deposit
×: a lot of snow deposit × ×: extremely much snow deposit

The finish of the present invention prevents amide oligomer from emitting on fiber surface during storage of polyamide fiber applied with the agent, and thus it contributes to preventing snow deposit and decreasing fluffs and ends down in down-stream process.

The finish of the present invention prevents not only amide oligomer but also urethane oligomer and polymer additives in polyurethane from emitting on the surface of polyamide-covered polyurethane yarn applied with the finish. And thus the finish contributes to decreasing snow generation in knitting process leading to improved knitting efficiency and knit fabric quality.

The finish of the present invention remarkably improves yarn cohesion in yarn production and down-stream processes, decreases fluffs and ends down, and enables to improve product quality and rationalize the processes. In other words, application of the finish of the present invention attains sufficient fiber cohesion of synthetic filament yarn, and enables to decrease or omit the interlacing steps in yarn production process.

## Claims

1. A fiber finish **characterized by** containing at least one compound selected from the group comprising urethane compounds produced in the reaction of polyhydric alcohol having 12 or more carbon atoms and organic diisocyanate, and amide compounds produced in the reaction of polycarboxylic acid having 12 or more carbon atoms and organic diisocyanate.

2. A fiber finish in Claim 1, which contains aliphatic ester and polyoxyethylene alkyl ether in addition to the said components.

3. A fiber finish in Claim 1, wherein the polyhydric alcohol having 12 or more carbon atoms is a dimeric alcohol of which molecular weight is 300 to 1,000.

4. A fiber finish in Claim 1, wherein the polycarboxylic acid having 12 or more carbon atoms is a dimeric acid of which molecular weight is 300 to 1,000.

5. A fiber finish in Claim 1, wherein the urethane compound is produced by reacting polyhydric alcohol having 12 or more carbon atoms and organic diisocyanate in an equivalent ratio of 1 to 2 - 10.

6. A fiber finish in Claim 1, wherein the amide compound is produced by reacting polycarboxylic acid having 12 or more carbon atoms and organic diisocyanate in an equivalent ratio of 1 to 2 - 10.

7. Synthetic fiber applied with the fiber finish in Claim 1.

8. Synthetic fiber in Claim 7, wherein the synthetic fiber comprises polyamide fiber, polyurethane fiber, or polyurethane yarn covered with polyamide fiber.

9. Application of one or more compounds selected from the group comprising urethane compounds produced by reacting polyhydric alcohol having 12 or more carbon atoms and organic diisocyanate, and amide compounds produced by reacting polycarboxylic acid having 12 or more carbon atoms and organic diisocyanate to a fiber finish.
